

Dec. 22, 1959

H. ROSS

2,917,798

METHOD AND APPARATUS FOR CASTING AND  
HANDLING FERRO-MANGANESE

Filed Dec. 2, 1957

2 Sheets-Sheet 1

FIG. 1.



FIG. 2.



INVENTOR

HALDON ROSS

BY

*Cushman, Darby & Cushman*

ATTORNEYS

Dec. 22, 1959

H. ROSS  
METHOD AND APPARATUS FOR CASTING AND  
HANDLING FERRO-MANGANESE

2,917,798

Filed Dec. 2, 1957

2 Sheets-Sheet 2

**FIG.3.**



**FIG.4.**



**FIG.5.**



**FIG.6.**



**FIG.7.**



**FIG.8.**



**FIG.9.**



INVENTOR  
HALDON ROSS

BY *Cushman, Darby & Cushman*  
ATTORNEYS

# United States Patent Office

2,917,798

Patented Dec. 22, 1959

1

2,917,798

## METHOD AND APPARATUS FOR CASTING AND HANDLING FERRO-MANGANESE

Haldon Ross, Rockwood, Tenn.

Application December 2, 1957, Serial No. 700,193

2 Claims. (Cl. 22—200)

This invention relates to the casting and handling of ferro-manganese and, in particular, relates to a method of casting ferro-manganese ingots and loading the ingots so cast on a transporting vehicle.

The casting and handling of ferro-manganese has heretofore been laborious. Methods used in casting of other type metals, such as, for example, pig iron, steel, or lead, are not adaptable to ferro-manganese casting procedures because molten ferro-manganese has a very high temperature, about 2900° F., and because ferro-manganese cracks or partially disintegrates in the cooling stage. Because of the peculiar characteristics of ferro-manganese, it has been common practice to cast ferro-manganese in a bed, and then break up the casting into small pieces and load the pieces into pans for subsequent transporting.

It is an object of this invention to provide a method of, and apparatus for, casting and loading ferro-manganese, which method and apparatus eliminate the need for breaking up a casting in order to transport it.

It is a further object of this invention to provide a method of, and apparatus for, casting and loading ferro-manganese which reduce the cost of equipment necessary for casting and loading operations and the time required for production.

It is a still further object of this invention to provide a method of, and apparatus for, casting ferro-manganese blocks, which method and apparatus decrease the number of beds required for casting ferro-manganese.

It is yet another object of this invention to provide a method of, and apparatus for, casting and loading ferro-manganese blocks, which method and apparatus provide for preparing the surface of a vehicle on which the blocks are to be loaded.

Still another object of this invention is to provide a method of, and apparatus for, casting and loading ferro-manganese blocks, which method and apparatus provide for a convenient means to lift the ferro-manganese blocks from the bed so that they may be loaded on a transporting vehicle.

Other objects and the advantages of this invention will become apparent when the following description is considered in conjunction with the annexed drawings, wherein:

Figure 1 is a plan view of a bed and transporting vehicle used for casting and handling ferro-manganese in accordance with the invention;

Figure 2 is a cross-sectional view taken on the line 2—2 of Figure 1;

Figure 3 is a side elevational view of a ferro-manganese block cast in accordance with this invention and being handled as provided by this invention;

Figure 4 is a plan view of a stool provided for handling the ferro-manganese;

Figure 5 is a side cross-sectional view of a stool such as is shown in Figure 4;

Figure 6 is a side view of a divider used in a ferro-manganese bed in accordance with this invention;

2

Figure 7 is an end view of a divider such as is shown in Figure 6;

Figure 8 is a side view of a fillet which may be used in a ferro-manganese bed in accordance with this invention; and

Figure 9 is an end view of a fillet such as is shown in Figure 8.

Another object of this invention is to provide a method of and apparatus for casting and molding ferro manganese blocks, which method and apparatus provides for casting beds having dimensions suitable for casting ferro manganese in accordance with this invention.

In the drawings the numeral 1 designates a bed area which may have any suitable foundation, such as, for example, an excavated area in the ground. The numeral 2 generally designates a single bed within the bed area 1. The bed comprises a plurality of side plates 3 joined end to end continuously so as to define a rectangular bed 2. Disposed within the bed are dividers 4, stools 5, and fillets 6.

As best shown in Figure 2, the floor of the bed comprises a layer of sand 7 over which is disposed a layer of cast iron blocks 8.

The numeral 9 designates a trough through which molten ferro-manganese is distributed to the bed area, and the numeral 10 designates a side trough, leading from the main trough 9. Through the trough 9 molten ferro-manganese is delivered to the bed 2. The numeral 11 designates a transporting vehicle which, as shown, is a flat top railroad car.

The dividers 4 are disposed in the bed 2 so as to divide it into sections 22, a fillet 6 is disposed at either end, and, as shown, two stools are disposed within each section.

Referring now more particularly to the components 35 of the bed, it will be noted that the side plates 3 are, as shown, rectangular in form. They are made of any suitable material, such as heat-resistant steel. It should be understood, however, that the side plates may be of any suitable shape without departing from the scope of the invention.

As best shown in Figure 6, the dividers have an elongated base portion 13 and an upwardly extending shank portion 14. At the top of the shank portion 14 is an eye 15 which is made, as shown, of a looped bar which extends through shank portion 14 into base portion 15. The components 13, 14 and 15 may be joined in any suitable manner, such as by welding or may be cast together. The base portion 13 of the dividers 4 is tapered to facilitate removal of blocks cast in the bed. By reference to Figure 2 it will be noted that the base portion 13 of the dividers is of less vertical height than the vertical height of the side plates 3. This feature is significant in that it allows for flow within a given bed, from section to section. It should be understood that a divider, as referred to in this application, refers to any structure which is used to separate a casting bed into sections. The hook 15, shown as connected with shank 14, facilitates movement of the divider by a crane.

Referring to Figures 4 and 5, it will be seen that the stools 5 have an enlarged disc-shaped base portion 16 above which is a tapering shank portion 17 that terminates at the base of a cylindrical portion 18. Carried at the top of the cylindrical portion 18 is a hook 19. The stools are made of any suitable material, such as heat-resistant steel, having a melting point higher than that of the metal to be cast. The term "stool" referred to in this application refers to any insert which may be used in accordance with this invention to aid in the loading of cast ingots on a transporting vehicle.

The fillets 6, as shown in detail in Figures 8 and 9, comprise a triangular base portion 20 into which are

secured hooks 21. The fillets 6 are not essential but are used to facilitate removal of a cast ingot from a casting section. As is apparent, there need only be two fillets used per bed, one at either end, because the tapering bases 13 of dividers 4 provide the taper between sections of the bed, except at either end. The fillets are also made of any suitable material, such as heat-resistant steel.

In carrying out the invention, a bed would be provided by first defining a bed area and then covering the surface of that area first with a layer of sand-fill, such as that designated by the numeral 7, and then with a layer of cast iron blocks, such as those designated by the numeral 8 in Figure 1. The side plates, such as those designated by the numeral 3, would be inserted so as to define a bed, and dividers 4 would be placed so that the bed 2 defined by the side plates 3 would be divided into sections. Fillets, such as those designated by the numeral 6, would be inserted at each end of the bed.

Because of the temperatures which are encountered when casting ferro manganese, the sections 22 of a bed should have certain minimum dimensions. The depth of a section should be one foot or more; one foot, four inches being the optimum minimum. This depth is measured from the top of blocks 8 to the top of side plates 3. The width of the section between defining side plates 3 should be five feet or more, six feet being the optimum minimum. The length of the section as measured between the outermost extension of adjacent base portions 13 should be five feet or more; five feet, four inches being the optimum minimum. Although the dimensions of the sections have critical minimum dimensions, there is no maximum limit, except that imposed by handling apparatus.

The exposed interior surfaces of the bed, that is, those which will come into contact with the molten ferro-manganese flowed into the bed through troughs 9 and 10, are coated with an aqueous mixture generally designated by the numeral 23. The mixture is preferably one consisting of water and lime or water and graphite.

#### Example 1

The beds were coated with a mixture of undissolved lime in a saturated solution of lime and water.

#### Example 2

The beds were coated with a mixture of undissolved graphite in a saturated solution of graphite and water.

The aqueous solution should be mixed so as to be of a nature that allows for application of the solution to the exposed interior surfaces of the bed by brush or of a nature that allows for application to those surfaces by spraying. The mixture used for the coating is not critical, but, of course, best results are obtained when all exposed surfaces are coated with a thin film. The coating prevents adherence of the ferro manganese to the components of the bed.

After the coating has been applied, molten ferro-manganese is flowed into the bed 2 through the troughs 9 and 10. Of course, the section nearest trough 10 fills first, however, as soon as filled to the level of the base 13 of the divider 4 separating that section from the next, the molten ferro-manganese spills over into the next section, and the process continues until all beds are filled to the level of the bases 13 of the dividers 4. After the beds are filled, preferably to this level or slightly above it, the flow of molten ferro-manganese to bed 2 is stopped. It should be understood that several side-by-side beds may be used and filled simultaneously. Of course, this allows the side plates between any two walls to serve as defining side plates of two beds at the same time.

After the beds are filled to the desired level, the metal is left to cool. This cooling period should be at least

one hour. During the cooling period, the metal will contract so as to draw away from the side plates and crack above the dividers.

After the cooling period has terminated, a hoist may be attached to the stools and the cast blocks 23 of ferro-manganese lifted from the sections, as shown in Figure 3.

It is usually desirable to transport the cast blocks to a stockpile. This is done by employing a transporting vehicle, such as that generally designated by the numeral 11, the surface of which has been prepared by covering the same with a layer of fire brick 26 on top of which is placed a layer of sand 27.

When it is desired to use the blocks 23 cast according to this invention, they are transported to the desired point. The stools 5 are easily removed from the blocks 23 because, as stated hereinabove, the ferro-manganese contracts while cooling, and draws away from the stools. Of course, the shape of the stools is such that even after contraction, the stools may be used for lifting purposes, i.e., they are provided with a tapering base comprising portions 16 and 17 (Figure 5).

Having thus set forth the invention, it is apparent that the objects above noted have been successfully achieved by this invention. Various modifications of the invention will become apparent to those of ordinary skill in the art after reading this disclosure. Therefore, it is intended that the matter contained in the foregoing description and the accompanying drawings be interpreted in an illustrative sense, and not in a limiting sense, when consideration is given to the appended claims.

I claim:

1. A new and improved method of casting and handling ferro-manganese in a bed having connecting side plates and containing stools, dividers, and fillets, said method including forming the bed with a flooring covered with a layer of sand, covering the sand with metal blocks, separating said bed into sections of predetermined dimensions with said dividers, placing at least one stool within each section, placing fillets at opposite ends of the bed to facilitate removal of a cast ingot from the bed, coating the internal exposed surfaces of the bed, treating the exposed surfaces of the stools and the exposed surfaces of the dividers with an aqueous mixture, flowing molten ferro-manganese into at least one of said sections, allowing the molten ferro-manganese to spill over the other sections until the sections are filled to at least a predetermined level and then allowing the molten metal to cool.
2. A new and improved method of casting and handling ferro-manganese as called for in claim 1 in which the aqueous mixture comprises a mixture of material selected from the group consisting of a mixture of lime and water and a mixture of graphite and water.

#### References Cited in the file of this patent

#### UNITED STATES PATENTS

|           |            |                |
|-----------|------------|----------------|
| 94,471    | Burt       | Sept. 7, 1869  |
| 278,512   | Critchlow  | May 29, 1883   |
| 387,174   | McCleane   | July 31, 1888  |
| 558,384   | Hainsworth | Apr. 14, 1896  |
| 609,671   | Hardy      | Aug. 23, 1898  |
| 735,596   | Sauveur    | Aug. 4, 1903   |
| 1,621,222 | Robertson  | Mar. 15, 1927  |
| 1,877,535 | Rosener    | Sept. 13, 1932 |
| 1,950,633 | Schmeller  | Mar. 13, 1934  |
| 2,051,413 | Barker     | Aug. 18, 1936  |
| 2,146,678 | Jung       | Feb. 7, 1939   |
| 2,480,899 | Bond       | Sept. 6, 1949  |

#### FOREIGN PATENTS

|       |               |               |
|-------|---------------|---------------|
| 5,367 | Great Britain | Nov. 14, 1883 |
|-------|---------------|---------------|